

June 21, 1949

**M. M. MARKS**

2,474,186

### REINFORCED CORE

Original Filed March 20, 1944



Inventor:  
Milton M. Marks;  
By Joseph O. Lange, Atty.

## UNITED STATES PATENT OFFICE

2,474,186

## REINFORCED CORE

Milton M. Marks, Chicago, Ill., assignor to Crane  
Co., Chicago, Ill., a corporation of Illinois

Substituted for application Serial No. 536,618,  
May 20, 1944. This application February 7,  
1947, Serial No. 727,024

1 Claim. (Cl. 22—165)

1

This application is filed in place of my abandoned patent application Serial Number 536,618, filed May 20, 1944.

This invention relates to cores for use in molds and is more particularly concerned with cores which must be structurally reinforced due to their particular shapes or sizes in order that they may not be readily broken before or after baking or while positioned in a mold during the pouring of the metal.

It has heretofore been common practice to apply embedded metal rods or arbors within cores for the purpose of reinforcing same, but this practice necessitates the removal of the reinforcing members from the cast products, which is often a relatively difficult operation when the reinforcing members are straight and even more difficult when such cast products are curved or have projections.

It is an object of this invention to provide an improved means and method for reinforcing cores, and consists essentially in the employment of reinforcing members formed of a material having suitable physical properties and which will withstand the temperatures employed in core baking and will subsequently melt and then burn or vaporize during the casting of a product to thereby leave a substantially clean vent passage for the escape of gases. It will thus be noted that reinforcing members of this type serve a dual purpose, as they strengthen or reinforce the core sufficiently to permit handling without breakage and further provide vent passages for the escape of gases generated during and after the pouring operation.

In the drawing:

Fig. 1 is a plan view illustrating the application of the improved reinforcing member to a sand core designed for use in casting a boiler section.

Fig. 2 is a sectional view taken along the line 2—2 of Fig. 1.

Referring now to the drawing for a better understanding of this invention, the sand core 6 is shown to illustrate a relatively fragile structure having side arms 7 and 8 and connecting end portions 9 and 11, all having relatively small cross-sectional areas and therefore normally requiring reinforcing members 12, 13, 14 and 16 in order to permit handling thereof without breakage. While a particular arrangement of reinforcing members has been shown as applied to one form of core, it should be understood that this is for illustrative purposes only in order to point out more clearly that any arrangement of reinforcing members within cores should contemplate

2

their dual uses as structural members and also as means for forming vent passages for gases generated during pouring as hereinafter described. The sand core structure 6 is shown with a pair of port openings 17 and 18 through which the generated gases may be vented during pouring, and it is therefore desirable to have the reinforcing members arranged to terminate at these openings, as shown.

10 The reinforcing members 12, 13, 14 and 16 are formed of material as hereinafter more specifically referred to, having the physical properties required to strengthen the core to permit handling of same without breakage. The material 15 must also be capable of withstanding the usual core baking temperatures without objectionable impairment of its physical properties, and further must be meltable and adapted for burning or vaporizing at temperatures created within the 20 core during the pouring of molten metal to thereby leave clean vent passages for the discharge of gases generated within the core. It will thus be noted that the type of material employed must necessarily be dependent upon the physical properties required for structural reinforcement purposes, the core baking temperature, and also upon the pouring temperature of the molten metal encountered. As an example of the type of material which may be employed in carrying out this 25 invention, certain thermoplastic materials, such as nylon, have been found to possess the desired physical properties even after being baked within a sand core, and then melt and either burn or vaporize when subjected to metal pouring temperatures to leave clean vent passages for the 30 discharge of generated gases.

The reinforcing strength of the plastic nylon is employed in the core during the course of baking and subsequently uses such property until 40 the molten metal is actually being poured. At the metal pouring temperature in the mold when such reinforcing of the core may be dispensed with, the nylon insert melts thereby imparting to the relatively complex hollow casting the benefits long 45 desired by industry; that is to say, there is no longer any worry about core wires being left in the hollow casting when the core sand is being removed. It is emphasized that the insert of this invention is not concerned with preventing the deformation of the surface of the core. This 50 is taken care of in the material of which the core itself is made. Thus there is no handicap encountered nor hardship assumed when the insert of this invention disintegrates during the 55 normal metal pouring mold temperatures.

Nylon possesses the desirable properties in that it will not melt at core baking temperatures, say at 450° F. but in excess of such temperatures, as for example those encountered in the mold during the pouring operation at a temperature of 2500° F. the nylon will disintegrate quite readily.

Thus it is easy to see that it reinforces and supports the core when desired to impart to it the necessary strength for handling during the assembly of the mold and withstanding the uplifting forces on the core by the molten metal acting underneath the core positioned in the mold during the pouring operation. It eliminates the more serious problem heretofore encountered of physically removing the reinforcing inserts heretofore used, such as metal wires for example, after the hollow casting has been made and it becomes necessary to remove the core therefrom. During a portion of the melting and subsequently during the metal cooling period this disintegration of the nylon insert serves to vent the core which constitutes an added advantage from the standpoint of improved foundry practice. The passage thus formed by the disintegration of the nylon serves as a vent to exhaust the gases generated by the burning of the core binding material, the evaporation of water and other volatile materials or gases present.

It is well known to those who are skilled in the art that the plastic nylon which is a generic term much as the terms wood and glass and is applied to the class of super polyamides, is produced either by the condensation of amino acids of the formula  $R-NH-R'-COOH$  where  $R'$  is a straight chain of at least five carbon atoms (U. S. Patent #2,071,253) or by the reaction of dibasic acids and diamines (U. S. Patent #2,130,523).

It is of interest to note that the nylon characterized as super polyamides of hexamethylene and adipic acid possesses the strength per unit weight in which the natural fibers are superior to the metals and is surpassed only by flax fibers.

Another unobvious benefit gained by this invention in employing nylon as the material for the core insert is that it is practically unaffected by

most organic acids, alcohols, halogenated hydrocarbons, cold dilute alkalies, soaps, ketones and organic solvent mixtures. In addition from a safety or health standpoint in handling the nylon insert by the core makers it is completely inert physiologically.

It will thus be seen in summarizing that reinforcing members formed of material as hereinbefore described may readily be shaped and positioned within sand cores during the core forming operation to add the desired strength thereto to permit handling without breakage, and also that the reinforcing members melt to leave clean vent passages of either straight or circuitous design to suit the requirements of the core design.

I claim:

10 A baked sand core of a shape requiring reinforcement, the said core having a reinforcing member imbedded therein formed of substantially rigid material consisting of a thermoplastic condensation product of the super polyamides class and possessing physical properties adapted to withstand core baking temperatures without disintegration but which will disintegrate at the temperatures encountered during the pouring of molten metal into a mold employing said reinforced core thereby to form substantially clear, unrestricted passages through the core for the venting of gases after the molten metal has been 20 25 30 poured.

MILTON M. MARKS.

#### REFERENCES CITED

The following references are of record in the 35 file of this patent:

#### UNITED STATES PATENTS

| Number    | Name   | Date          |
|-----------|--------|---------------|
| 982,670   | Hanson | Jan. 24, 1911 |
| 2,422,118 | Meyer  | June 10, 1947 |

#### OTHER REFERENCES

The Foundry, June 1946, page 136.